

# United States Patent

[11] 3,615,604

|      |                                                                                                                 |                                                                                                                                                                          |           |                                  |           |
|------|-----------------------------------------------------------------------------------------------------------------|--------------------------------------------------------------------------------------------------------------------------------------------------------------------------|-----------|----------------------------------|-----------|
| [72] | Inventors                                                                                                       | Friedrich-Wilhelm Kunitz<br>Leverkusen;<br>Willibald Pelz, Opladen; Erich Bockly,<br>Leverkusen, all of Germany; Agfa-Gevaert<br>Aktiengesellschaft, Leverkusen, Germany | [51]      | Int. Cl. ....                    | G03c 1/40 |
| [21] | Appl. No.                                                                                                       | 800,245                                                                                                                                                                  | [50]      | Field of Search.....             | 96/100    |
| [22] | Filed                                                                                                           | Feb. 18, 1969                                                                                                                                                            | [56]      | References Cited                 |           |
| [45] | Patented                                                                                                        | Oct. 26, 1971                                                                                                                                                            |           | UNITED STATES PATENTS            |           |
| [32] | Priority                                                                                                        | Mar. 2, 1968                                                                                                                                                             | 2,706,684 | 4/1955 Graham et al. ....        | 96/100    |
| [33] |                                                                                                                 | Germany                                                                                                                                                                  | 3,079,259 | 2/1963 Rauch et al. ....         | 96/100    |
| [31] |                                                                                                                 | P 16 22 920.2                                                                                                                                                            | 3,488,193 | 1/1970 Eynde et al. ....         | 96/100    |
| [54] | <b>SILVER HALIDE COLOR PHOTOGRAPHIC MATERIAL CONTAINING CYAN-FORMING COLOR COUPLER</b><br>4 Claims, No Drawings |                                                                                                                                                                          |           | Primary Examiner—J. Travis Brown |           |
| [52] | U.S. Cl. ....                                                                                                   | 96/100,<br>96/55                                                                                                                                                         |           | Attorney—Connolly and Hutz       |           |

**ABSTRACT:** Color couplers of novel structure that form cyan images in photographic silver halide emulsions and are highly stable as well as produce more stable and more light-fast images.

**SILVER HALIDE COLOR PHOTOGRAPHIC MATERIAL  
CONTAINING CYAN-FORMING COLOR COUPLER**

This invention relates to a process for the production of color photographic cyan partial images by color development and to a photographic material for carrying out the process.

In color photographic materials which are worked up to form color images by color-forming development, it is known to prepare the cyan part of the image from color couplers which are usually derivatives of phenols or naphthols. Although a large number of such cyan-forming couplers are known, no such cyan-forming couplers have yet been provided which ideally satisfy the many requirements which they have to meet. In fact, most color couplers have serious disadvantages. Inadequate stability of the residual coupler which has not been coupled with the color developer to form a dye image often causes discoloration of the whites of the images. The image dyes produced with oxidized color developer usually have unwanted side absorptions. Many dyes separate out in the form of a relatively coarse color grain whilst in others the coupling reaction proceeds too slowly. In general, the cyan dyes obtainable by color-forming development do not have sufficient fastness to light, satisfactory resistance to hydrolysis and the required stability to reducing agents.

It is the object of the present invention to provide cyan-forming couplers which are stable even under tropical conditions and which yield dyes which have high fastness to light and are stable under tropical conditions.

A photographic material comprising a red sensitive silver halide emulsion layer has now been found which contains cyan-forming couplers of the following formula which couplers on color-forming development yield cyan dyes of high stability and light-fastness even under tropical conditions:



in which

X is hydrogen or halogen such as chlorine or bromine;

R' and R'' are alkyl containing up to 18 carbon atoms, 45 Melting point 160-162° C.

preferably short-chain alkyl containing up to five atoms, e.g., methyl, ethyl or butyl, aryl, in particular phenyl, or aralkyl, in particular benzyl or phenylethyl, in which the phenyl groups may themselves be further substituted;

5 R''' is (1) alkyl, especially a short-chain alkyl group containing up to six carbon atoms, which alkyl groups are desirably substituted with aroxy groups, such as phenoxy groups the phenyl group of which may contain further substituents, especially alkyl containing up to 18 carbon atoms, halogen such as chlorine or bromine, alkoxy or nitrile; (2) an aryl group, e.g., phenyl or (3) an aralkyl group, e.g., benzyl or phenylethyl;

b hydrogen or the ring members required to complete a condensed benzene or tetrahydrobenzene ring.

15 The following couplers are, for example, suitable:



30 Melting point 162-164° C.





Melting point 154-155° C.



Melting point 76-78° C.

The color couplers according to the invention are prepared in known manner. The preparation of coupler 2 is described in detail below. Other couplers according to the invention are prepared in a similar way.

#### COUPLER 2

Stage 1. 103 g. of 5-nitro-2-amino-1,4-dimethoxybenzene were suspended in 400 ml. of pyridine. 134 g. of dimethyl aniline were added. 216 g. of p-(1,3, 3, trimethylpentyl)-phenoxyethyl chloroformate were added dropwise at room temperature with stirring, the temperature rising to 60° C. Stirring was then continued for 30 minutes without further supply of heat. The reaction mixture was poured while stirring into 3 liters of ice water and acidified to Congo Red with 5N HCL. The oil solidified. The crystals were separated by suction filtration, washed neutral with water and stirred up with about 2 liters of methanol, again separated by suction filtration and washed with methanol. The crude product was purified by recrystallization from 3 liters of n-propanol with the addition of active charcoal.

The yield was 152 g. of greenish yellow crystals of m.p. 147° to 149° C.

Stage 2. 152 g. of the nitro product produced in stage 1 were catalytically hydrogenated in 1.5 liters of tetrahydrofuran with Raney nickel at 50° C. and under 50 atmospheres excess pressure. The solution was filtered off from the Raney nickel and then concentrated by evaporation under vacuum (water-jet vacuum pump). The oily residue was stirred up with methanol, the oily amine then crystallized. The crystals were filtered off with suction and washed with methanol.

Yield: 128 g. of m.p. 99.5° to 101° C.

Stage 3. 87 g. of the amine produced in stage 2 and 52.8 g. of phenyl 1-hydroxy-2-naphthoate were melted and heated to 170°-175° C. in a vacuum, the phenol formed being distilled off. After heating during 45 minutes the hot melt was poured into 750 ml. of n-butanol. The precipitate was removed by suction filtration at room temperature and was washed with butanol. The crude product was recrystallized from 1.25 liters of butanol and washed with butanol and methanol. The yield was 111.5 g. of coupler 2 having a m.p. 160°-161° C.

The dye couplers according to the invention can be incorporated in a diffusion-fast form in the light-sensitive silver halide emulsion layers. This can be done in known manner by emulsifying the color couplers in the emulsion layer. Processes of this type have been known for a long time and can be easily employed in the present case.

According to one known method, the new compounds, if they are hydrophobic, are emulsified in a solvent with or without an oil-forming agent in gelatin and this emulsion is dried, allowed to swell again in water and then mixed with the silver halide emulsion. Other processes are known in which the color coupler is dissolved in an organic solvent and is directly mixed with the silver halide emulsion and in which the solvent is then evaporated off. The color couplers according to the invention are also suitable for use in this process. These



emulsions are then worked up to produce one-layered or multilayered materials on a support.

The new dye forming substances may be added not only to the light-sensitive silver halide emulsion itself but also to an adjacent insensitive layer. They may also be developed together with the color developer of the photographic material.

Any color-forming developers which contain a primary amino group may be used for development. It is especially desirable to use those of the p-phenylenediamine type, e.g., N,N-diethyl-p-phenylene diamine, N-monomethyl-p-phenylene diamine, N,N-dimethyl-p-phenylene diamine, 2-amino-5-diethylaminotoluene, N-butyl-N- $\omega$ -sulfonybutyl-p-phenylenediamine and the like.

Suitable binders for the layers are the known hydrophilic film-forming agents such as protein, especially gelatin, polyvinyl alcohol, polyvinyl pyrrolidone, cellulose derivatives such as carboxyalkyl cellulose, especially carboxymethyl cellulose, derivatives of alginic acid and their alkali metal salts or esters.

The cyan-forming couplers according to the invention are advantageously added to red sensitized photographic emulsions. Such emulsions may also contain the usual chemical sensitizers. These layers may in addition be stabilized by known additives, especially by the azaindene derivatives described in the publication by Birr in Z. wiss. Phot. 47 (1952) pages 2-28.

#### EXAMPLE 1

3 g. of the color coupler 6 are dissolved in 15 ml. of ethyl acetate at 55° to 60° C. and 3 g. of di-tert.-butyl phthalate are added. 50 ml. of 5 percent gelatin to which 8 g. of lauryl sulfate per kg. have been added as emulsifier are combined with the color coupler solution and intensively mixed for 10 minutes at 55° C. While this emulsion was still warm, 50 g. of a photographic silver bromide emulsion which had been prepared from 70 g. of AgNO<sub>3</sub> per kg. were added. The light sensitive mixture is diluted with 100 ml. of 7.5 percent gelatin solution and then applied in the usual manner to paper or a transparent support and is dried.

The photographic material produced in this way is developed in a color development bath of the following composition after exposure:

|                                |               |                 |
|--------------------------------|---------------|-----------------|
| N,N-diethyl-p-phenylenediamine | hydrochloride | 2.75 g.         |
| Sodium sulfite                 |               | 2 g.            |
| Potassium carbonate            |               | 75 g.           |
| Potassium bromide              |               | 0.5 g.          |
| Hydroxylamine hydrochloride    |               | 1.2 g.          |
| Sodium hexametaphosphate       |               | 1.0 g.          |
| Water                          |               | up to 1,000 ml. |

This material is then bleached, fixed and washed in the usual manner. A cyan dye image which has an absorption maximum at 678 m $\mu$  is obtained.

## EXAMPLE 2

3 g. of color coupler 4 are dissolved in 15 ml. of ethyl acetate at 55°-60° C. This solution is added to 50 ml. of 5 percent gelatin to which 8 g. of lauryl sulfate per kg. as emulsifier has been added, and this mixture is emulsified for 10 minutes at 55°-60° C. While this emulsion is still warm, 50 g. of the photographic silver bromide emulsion described in example 1 are added. The light-sensitive mixture is diluted with 100 ml. of 7.5 percent gelatin solution and then applied in the usual manner to paper or a transparent support and is dried.

After exposure and development in a developer described in example 1 and after the usual bleaching, fixing and washing, a cyan dye image which has its absorption maximum at 680 m $\mu$  is obtained.

The dye image may also be produced in the following developer after exposure.

|                                                                                              |                 |
|----------------------------------------------------------------------------------------------|-----------------|
| Benzyl alcohol                                                                               | 3.8 ml.         |
| Sodium hexametaphosphate                                                                     | 2 g.            |
| Sodium sulfite anhydrous                                                                     | 2 g.            |
| Sodium hydroxide 10%                                                                         | 5.5 ml.         |
| 4-Amino-N-ethyl-N-( $\beta$ -methanesulphonamidoethyl)-m-toluidine-sesquisulfate monohydrate | 5 g.            |
| Potassium bromide                                                                            | 1 g.            |
| Sodium carbonate monohydrate                                                                 | 50 g.           |
| Water                                                                                        | up to 1,000 ml. |
| pH at 21° C. 10.75                                                                           |                 |

After the usual bleaching, fixing and washing, a dye image which has the absorption maximum at 686 m $\mu$  is obtained.

We claim:

1. A silver halide emulsion which contains a cyan-forming color coupler of the following formula:



in which

X is hydrogen or halogen;  
 R' and R'' are alkyl containing up to five carbon atoms;  
 R''' is an alkyl group containing up to six carbon atoms  
 which group is substituted by a phenoxy group; and  
 the b's are the ring members required to complete a condensed benzene or tetrahydrobenzene ring.

5 2. An emulsion according to claim 1, wherein the phenoxy group is substituted with an alkyl group containing up to 18 carbon atoms.

10 3. An emulsion according to claim 1, wherein which contains a cyan-forming coupler of the following formula:



15 4. An emulsion according to claim 1, which contains a cyan-forming coupler of the following formula:



45

50

55

60

65

70

75